

Sept. 13, 1932.

F. J. TONE

1,877,541

JOINING ABRASIVE ARTICLES

Filed Feb. 13, 1929

*Fig. 1.*



*Fig. 2.*



*Fig. 4.*



*Fig. 3.*



INVENTOR

*Frank J. Tone*

*by Byers, Stebbins & Knobbe  
their attorneys*

## UNITED STATES PATENT OFFICE

FRANK J. TONE, OF NIAGARA FALLS, NEW YORK, ASSIGNOR TO THE CARBORUNDUM COMPANY, OF NIAGARA FALLS, NEW YORK, A CORPORATION OF PENNSYLVANIA

## JOINING ABRASIVE ARTICLES

Application filed February 13, 1929. Serial No. 339,511.

The present invention relates to joining abrasive articles, and more especially to a strong hot water resisting joint for segmental grinding wheels, such as pulp wheels, and to the method of making such joints. The general type of wheel to which the present invention most particularly relates is shown and claimed in my copending application Serial No. 252,468, filed February 7, 1928.

The joint can be formed by spraying the abutting faces of the abrasive blocks with molten metal and then filling the joint space with a low melting point metal which will flow in and complete the joint. A joint of such character is particularly desirable in pulp grinding wheels which have to operate in hot water.

Pulp grinding wheels are massive wheels which may be as large as five feet in diameter and four or five feet in length. It is not practicable to make wheels of such size from the artificially bonded abrasives which it is desirable to use for such purpose, as, for example, artificially bonded silicon carbide or aluminum oxide. It would be difficult, if not practically impossible, to make single-piece wheels of this size because of the difficulty in heating such large masses to a uniform temperature. Moreover, attempts to vitrify such large masses would result in producing structures with serious internal strains which might result in destruction of the wheel while in service. Any heat treatment required of such masses would be of excessive duration.

In making pulp wheels of artificially bonded abrasive, the practice has therefore been to build the wheels up from segments or blocks. These smaller segments can be readily molded, fired and annealed. The real problem is that of joining these segments together to meet the mechanical requirements of a massive pulp wheel used at the temperatures experienced in grinding pulp in the presence of hot water. The frictional heat generated in grinding the wood raises the temperature of the wheel and the pulp very near to the boiling point of water. Water is usually fed to the wheel so that the wheel

is subjected not only to heat, but also to the dissolving action of the hot water. The materials dissolved from the wood pulp in the water also add to the difficulties of the problem, since such materials are often erosive in their character.

Attempts have been made to form joints between the segments of pulp wheels, both using metal and various cements. When metal is used the segments have been mechanically secured to an interior arbor to support them against the grinding pressure and against centrifugal forces, and the metal which has been poured to fill up the crevices between the segments has been in the nature of a filler rather than a tensile strong segment-retaining joint. In forming wheels of this character a metal, such as lead, is poured into the crevices to fill them. The metal, while conforming somewhat to the irregular shape of the abrasive blocks, does not bond with them or form a strong tension resisting joint.

It has also been proposed to use cements based on phenolic condensation product resins. These cements when first applied form strong joints between the abrasive, but such joints lose their strength rapidly on being subjected to boiling water. It has been claimed that phenol condensation product resins when cured to the so-called "C" stage are infusible and insoluble in most solvents and unaffected by ordinary acid or alkaline solutions. I have found, however, that when such cements are employed in wheels subjected to boiling water, that they rapidly lose their strength. For example, I have found that a joint made of a phenolic condensation product resin cured to the "C" stage, with an initial tensile strength of about 1900 pounds per square inch, when subjected to boiling water for forty-eight hours dropped in strength to less than 200 pounds per square inch.

I have, however, developed a pulp grinding wheel having joints which are strongly bonded to the abrasive segments and which retain their strength even when subjected to hot water for long periods.

The preferred way of joining the segments

together is illustrated in the accompanying drawing, in which—

Figure 1 is a detail view showing a portion of the joint; and

Figures 2, 3 and 4 are side and top elevations and a cross-section, respectively, of a pulp wheel embodying the invention.

Referring to Figure 1 of the drawing, reference numerals 2 and 3 indicate abutting fragmentary portions of two segments united by the strong water-resisting joint indicated generally by reference numeral 4. The joint as illustrated comprises two thin layers of metal 5 and 6 applied into intimate contact with the surfaces of the abrasive blocks, and an intermediate layer 7 of a low melting point metal which is poured in and wets the metal facings 5 and 6. The abrasive segments or blocks may be of any suitable abrasive material, preferably molded blocks of artificially bonded abrasive having a high melting point bond. Examples of such abrasives are silicon carbide or aluminum oxide bonded by ceramic bonds vitrified at high temperatures. Such abrasive materials may have a tensile strength of 1,000 or more pounds per square inch.

The surfaces of the abrasive blocks are somewhat porous, showing fine pits between the abrasive grains and thus offering a good anchorage for the metal coating which is sprayed on.

The surfaces of the abrasive segments which are to be joined are first freed from dust and foreign particles by means of an air blast. They are then sprayed with molten metal, such as brass, to form the thin metal coatings 5 and 6 on the abrasive surfaces. The abrasive segments may be sprayed cold or may be heated preparatory to spraying. Devices for applying metal coatings by the molten spray process are well-known and do not need to be described in detail. See, for example, the book on "Metal Spraying" by Turner and Budgen, London, 1926, or article on "Metal Coating by Spraying Process" in "Handbook Encyclopedia of Engineering," New York, 1928. Usually the metal spray is produced by means of a metal wire which is fed through the nozzle of an oxy-acetylene torch. The metal is fused to a high temperature by the flame and is then carried by a high velocity stream of compressed air against the surface to be sprayed.

The sprayed metal is driven into the pores of the surface and into adherent contact therewith so as to wet or give the effect of wetting the surfaces of the abrasive segments. The coating of metal thus applied to the abrasive surface adheres to it strongly.

I have found that brass is a satisfactory metal to be sprayed in molten condition against the abrasive, since it wets or gives the effect of wetting the surface. Other

types of brasses and alloys may be employed, such as copper-zinc, copper-lead-tin, copper-lead-zinc, copper, and nickel alloys.

The segments are then gradually heated up to about 350° Fahrenheit, and after the application of a suitable flux have their metal-coated surfaces dipped into molten solder or other suitable metal at a temperature of about 500° Fahrenheit, sufficient to give the sprayed surfaces a thin coating of the solder or other metal. The segments are then in condition to be assembled in the wheel. It is, however, not necessary to follow the above procedure before assembling the segments into a wheel.

The segments are then assembled into wheel form, such as shown in Figures 2 and 3, by means of suitable assembling clamps and supports. In assembling the wheel small spacers are put between the segments so as to leave spaces between the adjacent metal sprayed surfaces to receive the metal which is cast into such spaces to form the joints. For example, as indicated in Figure 1, a small spacer or shim 8 may be put between the outside edges of the segments 2 and 3 to space them apart. Similar spacers will be placed between the inner edges of the segments in assembling the wheel. After the wheel is thus assembled, it is put into an oven at a temperature of about 300° Fahrenheit, which is then gradually increased to about 425° Fahrenheit in three or four hours. Solder or other suitable low melting point metal or alloy is then poured in between the metal-coated surfaces of the segments and the wheel is allowed to cool gradually. This solder is indicated at 7 in Figure 1. The edges of the joints to be filled with the metal are, of course, suitably stopped so as to retain the molten metal.

The solder or other metal wets the brass or coating metal so as to form a tensilely strong joint between the abrasive segments.

The bond or adherence between the metal joint thus formed and the abrasive surfaces is comparable in strength to the tensile strength of the abrasive material itself.

After the wheel is cooled down the spacers, such as those indicated at 8, are removed. The cavities left by the spacers may be filled with solder or other metal, or where the cavities left by the removal of the spacers are at the exterior of the wheel, the surface of the wheel may be dressed down to obliterate such cavities and form a continuous cylindrical surface.

The metal used for casting between the metal sprayed surfaces may be of any suitable low melting point metal, such as solder, lead, lead-tin, lead-bismuth, etc.

In Figures 2, 3 and 4 is illustrated a pulp wheel embodying the invention. The wheel is built up of a number of segments, indicated

by reference numerals 10, which are joined together by the strong hot water resisting joints 11, preferably formed as above described. The wheel is assembled as shown in Figures 2 and 3. In Figure 4 the wheel is shown as mounted on a suitable driving arbor or shaft 12 by means of end clamping plates 13 and 14.

Since the joints formed between the segments have a strength approximating that of the bonded abrasive, and since such joints retain their strength under working conditions, reliance may be placed upon the structural strength of such joints, and the elaborate precautions employed for securing the segments to a central drum or arbor in making pulp wheels which do not have such strong joints, may be obviated, thus reducing the cost of the wheel. So far as the strength of the wheel is concerned, a segmental wheel thus built up and formed is comparable to one of monolithic structure.

Tests have been made as to the strength of the metal joints formed, as above described, between sections of artificially bonded abrasive material. The metal joints showed initially a tensile strength of about 1,000 pounds per square inch, which is approximately that of the abrasive material itself. It was found that subjecting the joints to boiling water for prolonged periods did not decrease this strength. The strength of the metals in the joint is, of course, unaffected by the hot water, and the character of juncture between the metal and abrasive is such as to also be substantially unaffected by the hot water.

The joints of the character above described differ from those formed by merely pouring in a metal, such as solder or lead, between abrasive segments, in that such poured-in metal does not adhere strongly to the surface of the abrasive, as does the sprayed-on coating. The sprayed-on coating either wets or gives the effect of wetting the abrasive grains. The hot water, even containing the matters extracted from the pulp, finds nothing which it can attack or dissolve or emulsify in the metal joint as thus applied, thus differing from the joints formed from the phenol condensation product resins heretofore suggested for this purpose.

In forming the abrasive segments they are usually formed by tamping or pressing in shaping molds. The effect of so molding is to cause the outer skin of the segment in contact with the face of the mold to be somewhat more dense, compact and stronger than the interior of the segment. The composite joints formed of the sprayed-on and cast-in metal are therefore bonded with the strongest part of the segments and form, in effect, a supporting spider which strengthens the wheel. A wheel of this character formed of the built-up segments with such supporting strengthening spider may actually be safer

and stronger than would be a monolithic wheel. Moreover, since the joints are unaffected by the hot water, the strength of the wheel is not affected by its use in pulp grinding.

The metal joints as above described may be properly spoken of as cementitious joints since they serve to cement or secure the abrasive segments together against tensile forces, as contrasted with metal poured between the segments serving merely as a filler to fill up the inter-segment crevices.

I do not wish to limit myself as to the abrasive material. While the test-pieces referred to above are constituted mainly of fused alumina, I have made test wheels from bonded abrasive segments which were joined together with a form of joint resistant to boiling water.

While I have specifically illustrated and described the preferred embodiment of my invention, the invention is not so limited but may be otherwise embodied and practiced within the scope of the following claims.

I claim:

1. The method of uniting preformed blocks of abrasive material, which comprises spraying molten metal onto the faces to be united so as to form metal coatings firmly adherent to such surfaces, and uniting such metal-coated surfaces by metal cast between them and wetting and adhering to the metal coatings and while maintaining the metal coatings at a temperature below the temperature at which the metal flows.

2. The method of joining blocks of abrasive material, which comprises spraying molten metal against the surfaces to be united so as to form tightly adherent metal coatings thereon, heating the blocks, applying flux to the surfaces, dipping the surfaces in a low melting point metal, assembling the blocks to leave casting spaces between the thus metal-coated surfaces, and casting a low melting point metal into such spaces.

3. The method of making abrasive wheels for pulp grinding and the like, comprising forming a plurality of segments of abrasive material, spraying the surfaces of the segments to be united with molten brass so as to form tightly adherent brass coatings thereon, heating the segments to a temperature below the melting point of solder, and applying flux to the brass surfaces, coating the brass surfaces with a thin layer of solder, assembling the segments leaving crevices between the thus-coated surfaces, heating the thus-assembled wheel, and pouring molten solder into the crevices.

4. The method of joining molded abrasive blocks which comprises the steps of spraying the surfaces of the blocks to be joined with molten metal to force the metal into the surface pores of the abrasive blocks and thereby form adhering layers of metal on the sur-

faces of the blocks to be joined, and thereafter joining the blocks by applying a second metal between the metallic coated surfaces of the blocks, which second metal melts at a temperature below the temperature at which the metal coatings melt and which when melted adheres to the first metal coatings.

5. The method of joining two preformed abrasive blocks which comprises spraying molten brass against the surfaces of the blocks to be joined, and thereafter soldering the brass coated surfaces together.

10. An abrasive wheel consisting of a plurality of preformed abrasive blocks connected by bi-metallic joints, each of said joints comprising layers of higher melting point metal on the blocks and interlocked with said blocks by projections of said metal in the interstices thereof, and a layer of lower melting point metal connecting said higher melting point layers.

15. An abrasive wheel consisting of a plurality of preformed abrasive blocks held together by joints between said blocks consisting of a layer of solder between two layers of brass, each of said layers of brass being attached to an abrasive block by projections of the brass interlocking with the pores of the block.

20. In testimony whereof I have hereunto set my hand.

FRANK J. TONE.

35

40

45

50

55

60

65